

1

3,060,017

## HARD FACING ALLOYS

Arthur T. Cape, Monterey, Calif., assignor to Coast Metals, Inc., Little Ferry, N.J., a corporation of Delaware.

No Drawing. Filed June 7, 1961, Ser. No. 115,314  
1 Claim. (Cl. 75—128)

This invention relates generally to hard facing alloys and to hard castings, but has reference more particularly to improvements in the alloys described in my U.S. Patent No. 2,801,164.

In the aforesaid patent, an iron base alloy is described which consists of carbon in amounts of from about 1 to about 4.5%, chromium in amounts of from about 17% to about 27%, molybdenum in amounts of from about 4% to about 10%, cobalt in amounts of from about 5% to about 25%, and silicon in amounts up to about 4%, the remainder of the alloy being substantially all iron, and the alloy being substantially free of tungsten.

Although the aforesaid alloy has an exceptionally high hardness for the carbon-chromium range which it includes, the carbides in the alloy are of needle-like or needle-shaped form. Where the carbides are of this form or shape, there is a tendency for the carbides to grow or merge into each other, thus producing a continuous relatively brittle structure.

I have discovered that by incorporating relatively small amounts of nickel in the alloy, in the range of from about 1% to about 2% nickel, and preferably about 1.5%, the carbides in the alloy, instead of being of needle-like form or shape, assume the form of euhedral or well-shaped carbides. Where the carbides are in euhedral or well-shaped form, the carbides are discrete, and there are present in the structure of the alloy no continuous lines or planes of brittleness, so that the alloy resists wear to

2

a greater extent. These advantages become more apparent as the carbon content of the alloy increases.

The alloy, owing to this difference in the carbide structure, is able to withstand more severe impact than the material with the needle-like carbide structure.

In accordance with the invention, the alloys fall within the following ranges:

| 10         | Range    | Examples |      |      |      |
|------------|----------|----------|------|------|------|
|            |          | 1        | 2    | 3    | 4    |
| Carbon     | 1-4.5    | 4.25     | 4.25 | 1.25 | 1.75 |
| Chromium   | 17-27    | 23       | 23   | 23   | 23   |
| Molybdenum | 4-10     | 8        | 8    | 8    | 8    |
| Cobalt     | 5-25     | 10       | 10   | 10   | 10   |
| Nickel     | 1-2      | 1.5      | 1.5  | 1.5  | 1.5  |
| Silicon    | Up to 4% | .5       | 2    | .5   | .5   |
| Iron       | Balance  | Bal.     | Bal. | Bal. | Bal. |

It is to be understood that the expression "the remainder being substantially all iron," as used in the claim, is to be construed as including any other ingredients or impurities in relatively small or trace amounts, which are found associated with the various constituents of the alloy, as for example, manganese, sulphur and phosphorus.

25 Having thus described my invention, I claim:

An iron-base alloy consisting of carbon in amounts of from about 1 to about 4.5%, chromium in amounts of from about 17% to about 27%, molybdenum in amounts of from about 4% to about 10%, cobalt in amounts of from about 5% to about 25%, nickel in amounts of from about 1% to about 2%, and silicon in amounts up to about 4%, the remainder of the alloy being substantially all iron, said alloy characterized by the fact that the carbides in the alloy are of euhedral form.

35 No references cited.